

1

3,238,112

ELECTROPLATING OF METALS USING MERCAPTO-METAL COMPLEX SALTS

John H. Haslam, Landenberg, Pa., assignor to E. I. du Pont de Nemours and Company, Wilmington, Del., a corporation of Delaware

No Drawing. Filed July 3, 1962, Ser. No. 207,401

4 Claims. (Cl. 204—45)

This invention relates to compositions and processes for the electrodeposition of metals. It is more particularly directed to electroplating methods using baths containing mercapto compounds.

It has been found that plating baths containing mercapto compounds have a number of advantages not possessed by conventional plating baths. For example, the need for using such highly toxic substances as cyanide in the baths is eliminated. The baths give high efficiency, both at the anode and at the cathode. They can be used at high pH levels, with their attendant advantages. These baths have excellent throwing power, give a high quality plate, and have good conductivity. They also permit the use of copper and tin in their lower valence states, thereby saving plating current.

The mercapto compounds which can be used according to this invention are those of the formula



where

R is hydrogen, —COOH, an alkyl radical containing from 1 to 4 carbon atoms, or a hydroxylalkyl radical containing from 1 to 5 carbon atoms;

X is  $(\text{CH}_2\text{CH}_2\text{OH})_n$ ,  $(\text{CH}_2\text{CH}_2\text{NH}_2)_n$ , or  $(\text{CH}_2\text{CH}_2\text{COOH})_{n-1}$

where

R' is hydrogen, —COOH, a hydroxylalkyl radical containing from 1 to 4 carbon atoms, or an alkyl radical containing from 1 to 4 carbon atoms; and n is 1 or 2.

Preferred for use are

2-mercaptopropanol  
2-mercaptopropanol-2  
1-mercaptopropanol-2  
2-mercaptopropanol-3  
2-mercaptopropanol-4  
1-thioglycerol  
2-thioglycerol  
 $\alpha$ -Thiosorbitol  
Mercaptoacetic acid  
2-mercaptosuccinic acid  
Mercaptoethylamine

The metals which can be electrically deposited according to this invention are copper, tin, silver, gold, cadmium and zinc. Alloys of these metals, such as brass, can also be deposited. These metals can be deposited on such other metals as steel, copper and brass.

The electroplating bath is prepared by dissolving a conventional amount of a salt of the metal to be deposited in an aqueous solution of a mercapto compound which has been previously brought to pH 10-11 with a stoichiometric amount of sodium or potassium hydroxide. The mercapto compound should ordinarily be present at a concentration of from 2 to 20 moles per mole of the metal to be deposited. In the baths, the metals to be deposited are naturally present as salts with the mercapto compound. Excess sodium or potassium hydroxide in the bath generally improves plate quality and increases the conductivity of the bath. Conventional brightening

2

agents, such as Rochelle salts or sodium hydroxyacetate and other additives, can also be added if desired.

The plating is then carried out with conventional electroplating equipment, using ordinary electroplating techniques.

In order that this invention be better understood, the following examples are submitted:

Example 1

10 A solution of 45 grams of  $\text{SnCl}_2 \cdot 2\text{H}_2\text{O}$ , 90 milliliters of water and 10 milliliters of concentrated hydrochloric acid was prepared and then diluted to 500 milliliters and adjusted to pH 7 with sodium hydroxide. The resulting precipitate of stannous hydroxide which formed was filtered under vacuum and washed several times with distilled water to remove sodium chloride.

This precipitate was dissolved in a solution of 75 grams of 2-mercaptopropanol and 150 milliliters of water, previously adjusted to pH 10 with sodium hydroxide.

15 20 This solution was then diluted to 267 milliliters with water and placed in a Hull cell. Five grams of sodium hydroxide were added to the bath.

25 Steel plates were used as a cathode and a tin plate was used as an anode. These plates were immersed in the bath and a current of 1½ volts was passed through.

The resulting tin plate was matte-white. Both cathode and anode efficiency were 100%.

30 35 These steel plates were then brightened by dipping them into hot tallow, maintained at 207° C., for approximately 15 seconds.

40 This method can also be used to plate silver and gold on brass or copper by substituting 30 grams of  $\text{Ag}(\text{NO}_3)_2$  or 20 grams of  $\text{HAuCl}_4 \cdot 3\text{H}_2\text{O}$  for the  $\text{SnCl}_2 \cdot 2\text{H}_2\text{O}$ . The tallow treatment is omitted.

Example 2

An electroplating bath was prepared by dissolving 15 grams of cuprous oxide in a solution of 75 grams of mercaptoacetic acid in 150 milliliters of water, previously adjusted to pH 10 with sodium hydroxide.

45 This solution was then placed in a Hull cell, 10 grams of sodium hydroxide were added, and the resulting bath was used to electroplate copper on steel, using a copper anode and a current of 2½ volts and 1 ampere.

The resulting copper was bright and attractive over the whole current density range.

50 Mercaptoethylamine can be substituted for mercaptoacetic acid in this process, in equivalent amounts, with similar results.

Example 3

55 A solution of 20 grams of 1-thioglycerol and 20 milliliters of water was adjusted to pH 10 with sodium hydroxide. Ten grams of cadmium oxide were then added to this solution in small quantities and the whole was made up to 267 milliliters with water.

60 65 This solution was then placed in a Hull cell, 5 grams of sodium hydroxide were added, and the bath was electrolyzed using a steel cathode, a cadmium anode and a current of 0.5 ampere and 1 volt. The resulting plate was bright and the anode and cathode plating efficiencies were essentially 100%.

Example 4

70 75 Eight grams of  $\text{ZnO}$  were dissolved in 200 milliliters of water, and sodium hydroxide was added until the pH of the solution was 9. The resulting precipitate was filtered and washed with water.

This precipitate was then dissolved in a solution of 200 milliliters of water and 25 grams of 2-mercaptopropanol. The pH of this solution was adjusted to 10 with sodium

hydroxide and the solution was then made to 267 milliliters with water.

This solution was used as an electroplating bath, using a steel cathode, a zinc anode and a current of 0.5 ampere and 5 volts.

The resulting zinc plate was bright in the intermediate current density range.

The embodiments of the invention in which an exclusive property or privilege is claimed are:

1. An improved electroplating bath consisting essentially of an aqueous solution of a metal salt of a compound of the formula



where

R is selected from the group consisting of hydrogen, —COOH, alkyl radicals containing from 1 to 4 carbon atoms, and hydroxyalkyl radicals containing from 1 to 5 carbon atoms; and

X is selected from the group consisting of (CHR')<sub>n</sub>OH, (CHR')<sub>n</sub>NH<sub>2</sub>, and (CHR')<sub>n-1</sub>COOH

where

R' is selected from the group consisting of hydrogen, —COOH, hydroxyalkyl radicals containing from 1 to 4 carbon atoms and alkyl radicals containing from 1 to 4 carbon atoms; and

n is a whole positive number less than 3

the metal in said salt being selected from the group consisting of tin, copper, silver, gold, cadmium and zinc.

2. An electroplating bath consisting essentially of an aqueous solution of a 2-mercaptopropanoic acid salt of a metal selected from the group consisting of tin, copper, silver, gold, cadmium and zinc.

3. A method for the electrodeposition of tin, copper, silver, gold, cadmium and zinc, said method comprising passing an electric current from a suitable anode to a cathode to be plated, through an aqueous bath consisting essen-

tially of an aqueous solution of a metal salt of a compound of the formula



where

R is selected from the group consisting of hydrogen, —COOH, alkyl radicals containing from 1 to 4 carbon atoms, and hydroxyalkyl radicals containing from 1 to 5 carbon atoms; and

X is selected from the group consisting of (CHR')<sub>n</sub>OH, (CHR')<sub>n</sub>NH<sub>2</sub>, and (CHR')<sub>n-1</sub>COOH

where

R' is selected from the group consisting of hydrogen, —COOH, hydroxyalkyl radicals containing from 1 to 4 carbon atoms and alkyl radicals containing from 1 to 4 carbon atoms; and

n is a whole positive number less than 3

20 the metal in said salt being selected from the group consisting of tin, copper, silver, gold, cadmium and zinc.

4. A method for the electrodeposition of tin, copper, silver, gold, cadmium and zinc, said method comprising

25 passing an electric current from a suitable anode to a cathode to be plated, through an aqueous bath consisting essentially of a 2-mercaptopropanoic acid salt of the metal to be thus deposited.

#### References Cited by the Examiner

##### UNITED STATES PATENTS

- |           |        |                      |          |
|-----------|--------|----------------------|----------|
| 1,857,507 | 5/1932 | Hichman et al. ----- | 204—46   |
| 2,113,517 | 4/1938 | Powell et al. -----  | 204—46   |
| 2,495,668 | 1/1950 | Wilson et al. -----  | 204—52.1 |

##### FOREIGN PATENTS

- 690,978 4/1953 Great Britain.

JOHN H. MACK, Primary Examiner.

JOHN R. SPECK, Examiner.